

Feb. 24, 1925.

A. J. LEWANDOWSKI ET AL

1,527,521

MOLD FOR CASTING INGOTS

Filed Jan. 10, 1923

FIG. 1.



FIG. 2.



FIG. 3.



FIG. 4.



Witness

Edwin L. Bradford

Adam J. Lewandowski,  
And Salvador Polito,  
By M. C. Dyre,  
Attorney

## UNITED STATES PATENT OFFICE.

ADAM J. LEWANDOWSKI AND SALVADOR POLITICO, OF PORT HURON, MICHIGAN; SAID POLITICO ASSIGNOR TO SAID LEWANDOWSKI.

## MOLD FOR CASTING INGOTS.

Application filed January 10, 1923. Serial No. 611,774.

To all whom it may concern:

Be it known that we, ADAM J. LEWANDOWSKI and SALVADOR POLITICO, citizens of the United States, residing at Port Huron, in the county of Saint Clair and State of Michigan, have invented certain new and useful Improvements in Molds for Casting Ingots; and we do hereby declare the following to be a full, clear, and exact description 10 of the invention, such as will enable others skilled in the art to which it appertains to make and use the same.

This invention relates to casting molds generally and more particularly to an improved mold for casting brass billets.

The general practice in casting billets in most foundries prior to the present time is to employ molds about four feet long which are split longitudinally, so that they can be 20 opened to permit the removal of the billets. Three rings are usually employed with each of these molds, and these rings surround the mold and are fastened with wedges. When the mold is filled with hot metal, the metal 25 nearest the sides of the mold becomes cooled before the metal at the center, and this central metal will remain hot for a considerable length of time and shrink, and owing to this the central portion of the billet has to be 30 supplied with molten metal until the shrinking discontinues. This procedure leaves a rough top on the billet which has to be cut off before the billet is used, and for this reason the mold has to be longer than the length 35 of the finished billet. In the usual method, one end is cut off from the billet and then the billet is cut in two pieces, each of which forms a billet in itself. The piece of waste material cut from the end of the billet 40 weighs about twenty-five pounds and it must be remelted in order to be utilized. The mold provided by the present invention forms a solid billet having no waste portions. Owing to the present construction 45 the metal will shrink evenly all around and an even surface will remain at the top of the billet after the same has been cast. This has been found to be the case from actual practice and the use of the present mold will 50 eliminate sawing the billet.

The mold forming the subject-matter of the present invention is of simple and inexpensive construction and in use it will save time and labor and eliminate the necessity of

removing waste portions from the billet. 55 The billet formed by the present mold is ready for the road mill as soon as it is removed from the mold, and the billet will not contain blow-holes or cavities.

From the foregoing it will be understood 60 that it is the primary object of the present invention to provide a novel mold capable of producing billets free from piping and blow-holes and of solid structure throughout.

With the foregoing object outlined and with other objects in view which will appear as the description proceeds, the invention consists in the novel features herein-after described in detail, illustrated in the 70 accompanying drawing and more particularly pointed out in the appended claims.

Referring to the drawings:

Figure 1 is a perspective view of the improved mold with the cover in open position.

Fig. 2 is an enlarged vertical sectional view of the same with the cover closed.

Fig. 3 is a perspective view of the base portion of the mold.

Fig. 4 is a side view partly in vertical section of a portion of a billet and the mold base, illustrating the manner in which the billet is keyed to the base during pouring.

In the drawing, 1 designates a base of 85 any suitable construction and preferably formed of cast iron provided with bolt holes 2 to facilitate bolting or anchoring the base to a suitable foundation. The base is preferably provided with an upwardly extending integral substantially cylindrical portion 3 provided at one side with a dovetail recess 4, the upper end of which is of smaller area than the lower end.

A mold body 5 preferably of cylindrical shape and made of a single piece of cast iron rests on the base 1 and has a bore 6 of tapered or frusto-conical shape, the lower portion of which snugly engages the circular surface of the cylinder 3. The upper end of the bore 6 is of less area than its lower end in order that the body 5 may be raised off of the base and off of the billet cast by the mold, and this upper end of the bore has its surface merging into a horizontal annular shoulder 7, which merges into a cylindrical surface 8, that is of greater diameter than the bore 6. The shoulder 7 and cylindrical

surface 8 form a pocket to receive the feeding ring 9. This feeding ring preferably includes a cast iron collar 10 having an inwardly extending flange 11 at its lower end, 5 which rests on the shoulder 7. This collar is provided with a lining 12 adapted to aid in preventing too rapid cooling of the molten metal at the upper end of the mold, and it is to be noted that the bore 13 of the 10 lining forms a continuation of the surface of the bore 6, so that the metal may readily flow through the bore of the lining into the bore of the body 5.

Arranged at the upper end of the body 5 15 is a cover 14 preferably connected to the body by means of a hinge 15 and having a lining 16 designed to close the bore of the ring 9 and also aid in preventing too rapid cooling of the molten metal within the upper 20 end of the body 5. The linings 12 and 16 are preferably formed of a composition including three parts of asbestos, one part of kaolin clay, one part of silica soda and water, and it has been found in practice 25 that this composition will last for about one hundred operations, that is, for about one hundred charges in the mold. When the lining loses its efficiency, it may be readily replaced, and to facilitate re-lining the collar 10, said collar is preferably removable 30 from the body of the mold.

In operation, the inner surface of the bores 6 and 13, and the upper surface of the member 3, are washed with plumbago and oil 35 before pouring the metal, and this will permit the mold to slide easily off the billet and leave the bores smooth. This washing will also facilitate the removing of the billet from the base. After pouring the mold full 40 of hot metal and closing the cover for about five minutes, which is about the time required before metal on the top becomes hard, the metal then will be about one and one-half inches lower in the mold than when it 45 was poured, the one and one-half inches representing the shrinkage which has taken place during the cooling of the metal. Owing to the linings 12 and 16, the heat from the metal at the upper portion of the mold 50 will not be dissipated as rapidly as that in the metal below the ring 9, and consequently as the metal below said ring cools and shrinks, the molten metal above will automatically descend into the cavities formed by the 55 shrinkage and will thus prevent blow-holes and piping.

The lower portion of a billet 17 is shown in Figure 4 and it will be seen that the metal during pouring will enter the recess 60 4 and form a lug 18 that functions to key the billet to the member 3. This key prevents the billet from rising when the mold body 5 is raised upwardly off of the billet. After the body of the mold is raised, the 65 billet may be detached by moving the billet

in the direction of the arrow 19, and this will cause the lug 18 to detach itself from the recess 4. Subsequently the lug 18 may be detached from the billet by striking said lug with a hammer or the like. 70

The upper end of the mold body is provided with diametrically opposite notches 20 to receive the tongues used in stripping the mold body from the ingot. Recesses 21 are also arranged at the upper end of the 75 mold body to receive a tool employed in removing the ring 10 from the mold body.

From the foregoing it is believed that the construction, operation and advantages of 80 the invention may be readily understood and it is apparent that various changes may be made in the construction disclosed, without departing from the spirit of the invention as expressed in the claims.

What is claimed and desired to be secured 85 by Letters-Patent is:

1. A mold including a base provided with a vertical extension having a key recess at one end of its edges provided at its upper end with a reduced portion, and a hollow 90 mold body resting on said base and surrounding said extension, said recess communicating with the interior of said mold body to permit molten metal poured in the mold body to flow into the recess and key a cast billet to said base against axial movement but permitting the detachment of the billet from the base when the billet is moved in a direction perpendicular to the axis of the 95 billet. 100

2. A mold including a base provided with an upwardly extending portion having a key recess at its edge provided at its upper end with a reduced portion, and a mold body resting on said base and having a bore tapered from bottom to top, the outer surface of the upwardly extended portion of the base snugly engaging the surface of said bore, and said bore communicating with said recess to permit molten metal poured in the bore of said mold body to flow into said recess and thus key a cast billet to the base against axial movement while the mold body is being stripped from the billet. 110

3. A mold including a hollow body portion having a base closing the lower end of its bore, a lining ring of heat insulating material arranged at the upper portion of said bore, and a cover for closing the upper end of the bore of said ring and provided with a lining of heat insulating material adapted to snugly engage the upper end of said ring and maintain metal in the bore of the ring in heated condition for a relatively great length of time. 115 120

4. In a mold, a hollow body portion, a heat insulating annulus forming the inner surface of the upper portion of the bore of said body, and a cover provided with a heat insulating lining designed to snugly 130

engage the upper edge of the heat insulating annulus and close the upper end of the bore of said body portion.

5. The combination with a mold having a bore, of a metal ring arranged within the body portion, and an annulus of heat insulating material arranged within said ring and located at one end of said bore, the surface of the bore of said annulus forming 10 a continuation of the surface of the bore of the body portion.

6. A mold including a body portion having a bore, said bore including a portion tapered from bottom to top, the upper end 15 of the tapered portion merging into a shoulder, and an enlarged cylindrical surface also merging into said shoulder, a ring engaging said cylindrical portion and having a flange at its lower end resting on said 20 shoulder, and an annulus of heat insulating material arranged within said ring and having the surface of its bore forming a continuation of the tapered surface of the bore of the mold body.

25 7. A mold including a body portion having a bore, an annulus of heat insulating material arranged at the upper end of said

bore, said annulus being formed of a composition including substantially three parts of asbestos, one part kaolin clay, one part 30 silica soda and water.

8. A mold including a base provided with an upwardly extending portion, a body resting on said base and having a bore, the surface of the lower portion of which engages the outer surface of said upwardly extending portion, a removable metal ring arranged at the upper end of the body portion, an annulus of heat insulating material carried by said ring and having a surface 40 of its bore forming a continuation of the surface of the bore of the body portion, and a cover for closing the upper end of said bores provided with a lining of heat insulating material.

45 In testimony whereof we affix our signatures in presence of two subscribing witnesses.

ADAM J. LEWANDOWSKI.  
SALVADOR POLITICO.

Witnesses:

WILLIAM J. POWELL,  
JOHN R. GANLIS.